

Nov. 27, 1928.

1,693,067

H. H. WILLIAMS

MAKING HUBS

Filed May 12, 1926

2 Sheets-Sheet 1



Inventor

HERBERT H. WILLIAMS.

By His Attorney

Anthony Mina

Nov. 27, 1928.

1,693,067

H. H. WILLIAMS

MAKING HUBS

Filed May 12, 1926

2 Sheets-Sheet 2



Inventor

HERBERT H. WILLIAMS.

By his attorney

D. Anthony Meira

Patented Nov. 27, 1928.

1,693,067

# UNITED STATES PATENT OFFICE.

HERBERT H. WILLIAMS, OF BROOKLYN, NEW YORK, ASSIGNOR TO THOMAS E. MURRAY,  
OF BROOKLYN, NEW YORK.

## MAKING HUBS.

Application filed May 12, 1926. Serial No. 108,448.

The invention relates to vehicle hubs and similar hollow articles, and facilitates their production at a comparatively low cost in labor and material, and has other advantages referred to in detail hereinafter. The accompanying drawings illustrate embodiments of the invention.

Figs. 1 and 2 are respectively a side and an end view of a segmental formed blank; 10 Figs. 3 and 4 are respectively a longitudinal section and an end view of two formed blanks assembled for welding;

Figs. 5 and 6 are respectively a side elevation and a cross section on the line 6—6 of 15 Fig. 5, of the welded product;

Fig. 7 is a similar section of the finished product;

Figs. 8 and 9 are respectively an end and a side view of the rolled bar stock from which 20 the segments are made;

Fig. 10 is a side elevation of the roughly finished product;

Fig. 11 is a similar view of a different design;

Fig. 12 is a longitudinal half section showing the product ready for use.

The hub (referring first to Fig. 10) has cylindrical portions 1 and 2 of different diameters with a wide annular flange 3 to which 25 the wheel is bolted or otherwise secured and generally has one or more internal annular shoulders 4 and ribs 5. In the design of Fig. 11 there are cylindrical portions 6 and 7, an outer annular flange 8 and ribs 9 and 10; 30 this being of the same character as the hub of Fig. 11 and differing only in design.

The forged welded product described is turned to the shape shown in full lines, Fig. 12; the dotted lines corresponding to Fig. 10. 40 The outer face of the smaller tube 1 is turned as at 1<sup>a</sup> and reduced on the end as at 1<sup>b</sup> to receive the wheel and fastening devices, and the flange 3 is turned on the flat face 3<sup>a</sup> for attachment to the wheel. The insides of the tubes are turned as at 1<sup>c</sup> and 2<sup>a</sup> and the ends 45 are squared off at 1<sup>d</sup> and 2<sup>b</sup>. It is not necessary in all cases to do all of the turning described. One of the advantages of this invention is that the hub may be shaped in some cases to eliminate part of the machine operations and in all cases to reduce the amount of machine work.

The hub is produced by forging separate segments and welding these together. In 50 making the hub of Fig. 10, the segments are

forged to the shape shown in Figs. 1 and 2 having tubular portions of different diameter, 11 and 12 between which is an annular flange 13 and within which are shoulders 14 and 15 and a rib 16 which forms a stop for a bearing pressed into the left end of the hub. 60 By the shoulders 14 and 15 the thickness of the tubular wall is maintained approximately constant throughout the length. The segment is substantially semi-circular with an 65 extension 17 on each of the longitudinal edges to be taken up in the welding. Two such forgings are assembled between positive and negative electrodes 18 and 19 shaped to fit them closely and are brought together with 70 their extended edges in contact and welded preferably by the method of the Murray Re-issue Patent No. 15,466 of October 10, 1922 in which while the parts are pressed together 75 a current of extremely high density is passed across the joint for a very brief period of time. As a result the surplus stock 17 is extruded sidewise forming fins 20 as in Figs. 5 and 6. The extruded metal or "flash" is removed by cutting or grinding it off, leaving 80 the finished section as in Fig. 7 and the external appearance as in Fig. 10. The rough welded hub is then turned down as in Fig. 12 or otherwise shaped to form the accurate cylindrical and flat surfaces required for attachment of the wheel to the outside and of the shaft and bearing to the inside.

The segments can be economically produced from rolled steel bar stock, the cross section of which corresponds approximately 90 to the longitudinal section of the hub. For example, for segments like Fig. 1 we may use the bar stock of Figs. 8 and 9 having flat portions 21 and 22 in different planes with a longitudinal flange 23 on one side and with 95 shoulders 24 and 25 and a longitudinal flange 26 on the other side. Starting with such bar stock the forging operations are reduced and a saving in material is effected compared with the ordinary forging from plain blanks.

For making the hub Fig. 11, the process would be substantially the same, starting with a piece of rolled bar stock corresponding approximately with the longitudinal section of the hub, forging the segments, welding and trimming off the flash and finally turning to exact dimensions.

By this method, the parts may be produced of a strength equal to or greater than by ordinary methods of manufacture and at the 110

same time with a substantial reduction in weight. By forging the article in segments the material may be distributed to the best advantage to secure strength and lightness.

- 5 5. Intricate shapes and sections not otherwise possible in a one-piece forging may be produced, thus permitting a freedom of design not obtainable by other methods. By the Murray method of welding described, the  
10 article can be made as strong at the joint as elsewhere, giving in effect a one-piece forging which is cheaper and capable of greater variation in design than any forgings heretofore available.  
15 6. The original stock and the segments forged therefrom should be of proper dimensions to allow surplus stock entirely over the faces which are to be turned down in the final operation. And this turning operation may  
20 be supplemented or substituted by grinding and other known methods of working to exact dimensions. Various other articles of tubular shape with annular flanges and shoulders may be made by the same method,  
25 7. providing a surplus of metal wherever the dimensions are to be accurately produced by turning or similar operations.

Various modifications may be made by those skilled in the art without departing  
30 from the invention as defined in the following claims.

What I claim is:

- 35 1. In the production of vehicle hubs or similar hollow articles the method which consists in cutting blanks from a rolled bar having flat portions extending lengthwise in different planes and a longitudinal flange on one side, forging such blanks into segments

having cylindrical ends of different diameters formed from the flat portions of the blank and an outer annular flange formed from the longitudinal flange of the blank, welding such segments together along their longitudinal edges with a resistance weld, trimming off the flash produced at the joints and turning the rough product thus formed to the exact dimensions desired. 40

2. In the production of vehicle hubs or similar hollow articles the method which consists in cutting blanks from a rolled bar having flat portions extending lengthwise in different planes and a longitudinal flange on one side, forging such blanks into segments having cylindrical ends of different diameters formed from the flat portions of the blank and an outer annular flange formed from the longitudinal flange of the blank and welding such segments together along their longitudinal edges. 45 50

3. In the production of vehicle hubs or similar hollow articles the method which consists in cutting blanks from a rolled bar having flat portions 21 and 22 extending lengthwise in different planes and a longitudinal flange 23 on one side at the junction of said flat portions, forging such blanks into segments having cylindrical ends of different diameters formed from the flat portions of the blank and an outer annular flange at the junction of said cylindrical portions formed from the longitudinal flange of the blank and welding such segments together along their longitudinal edges. 55 60 65 70

In witness whereof, I have hereunto signed my name.

HERBERT H. WILLIAMS.